

1

2,938,775

HYDROCARBON OILS CONTAINING ASHLESS  
DISPERSANT INHIBITORSJoel R. Siegel, Irvington, N.J., assignor to Esso Research  
and Engineering Company, a corporation of Delaware

No Drawing. Filed Dec. 6, 1956, Ser. No. 626,590

6 Claims. (Cl. 44—62)

The present invention is directed to the stabilization of hydrocarbon oils and particularly of petroleum distillates against discoloration and the formation of sediment during storage. More particularly, the invention concerns the stabilization of hydrocarbon fuel oils during storage by incorporating into the oils addition agents that inhibit degradation of the fuel oils and which at the same time serve to disperse any sediment producing materials that may have formed in the fuel oil. These addition agents are of particular value because they do not form ash or residues when the fuel oils are burned.

The hydrocarbon fuel oils with which this invention is particularly concerned broadly comprise petroleum distillates that are commonly employed in various burner systems, as fuels for diesel engines, as jet fuels and as domestic or industrial heating oils. These fuel oils may be generally characterized as those that consist of a major proportion of hydrocarbons boiling in the range of from about 350° F. to about 900° F. It is common practice to incorporate cracked hydrocarbon stocks in such fuel oils, and this practice aggravates the tendency of the fuel oils to form sediment on storage. It has been found that if 10 percent or more of the fuel oil composition comprises cracked stocks, the formation of sludge or sediment during storage may be markedly increased, leading to the plugging or fouling of oil lines, filters and burner nozzles.

Attempts have been made in the past to overcome the sediment-forming problem by incorporating in the fuel oils various addition agents, some of which have met with a degree of success. Many of these additives, however, particularly metal salts such as metal naphthenates, metal sulfonates and metal salts of alkyl phenol sulfides, have been objectionable in that they leave an ash residue on combustion.

It is a primary object of this invention to improve the stability of petroleum hydrocarbon fuel oils against the formation and precipitation of sediment while at the same time minimizing the formation of ash when such fuels are burned. It is an additional object of the invention to improve the color stability of such fuel oils.

It is still a further object of this invention to provide improved addition agents, and improved methods of preparation of the same, for accomplishing the objects stated above.

In accordance with the present invention, the sediment-forming tendencies of petroleum hydrocarbon oils, and particularly of fuel oils, can be markedly reduced by incorporating therein minor proportions, of the order of from about 0.001% to about 0.2%, of a polymeric material containing an azomethine linkage. The polymeric materials of this invention are preferably prepared by copolymerizing a mixture of three types of monomeric materials, namely, a long chain alcohol ester of a conjugated unsaturated dibasic acid, a vinyl ester of a short chain fatty acid and an alpha beta unsaturated aldehyde or ketone, and then reacting the resulting copolymer with a long chain tertiary alkyl primary amine. Suitable

2

vinyl esters include vinyl acetate and vinyl propionate. The dibasic acid ester may be a maleate, fumarate, itaconate, aconitate, or the like.

The dibasic acid ester component of the copolymer is 5 preferably an ester of fumaric acid or of mixed fumaric and maleic acids and a long chain alcohol of from about 8 to 24 carbon atoms such as octyl (C<sub>8</sub>), lauryl (C<sub>12</sub>), tridecyl (C<sub>13</sub>), arachidyl (C<sub>20</sub>), behenyl (C<sub>22</sub>), or tallow (C<sub>16-18</sub>) alcohols produced by the hydrogenation of tallow acids. The alpha beta unsaturated aldehyde or ketone 10 is one having the general structure:



15 wherein R is selected from the class consisting of hydrogen, aliphatic groups of from 1 to 8 carbon atoms, phenyl groups and alkyl phenyl groups of from 1 to 3 alkyl carbon atoms, and R' and R'' are selected from the class 20 consisting of hydrogen and aliphatic groups of from 1 to 3 carbon atoms. Among the aldehydes or ketones that may be employed are included acrolein, cinnamaldehyde, benzalacetone and methyl vinyl ketone.

25 Preferably the copolymers are prepared from mixtures of the monomers in the proportion of about 1 to 1.5 moles of vinyl ester, about 0.5 to 0.7 mole of dibasic acid ester and about 0.3 to 0.5 mole of the aldehyde or ketone. The polymerization is conducted in a solution of benzene or other solvent, e.g., xylene, toluene, etc. 30 (50 percent by weight) at temperatures of 60° to 212° F. and may be promoted by gamma radiation or by use of a peroxide type catalyst such as benzoyl peroxide, a hydroperoxide or an azo catalyst such as alpha-alpha'-azo-bis-iso-butyronitrile. The polymerization is conducted until a product of 1000 to 100,000 but preferably 2000 to 20,000 Staudinger molecular weight is produced.

35 The copolymer product after boiling off the solvent is then reacted with a long chain tertiary alkyl amine by mixing the product with from 1 to 3 moles, preferably 1.25-2.5 moles of amine per mole of aldehyde or keto group in the copolymer, the mixture being dissolved in some suitable non-aqueous high boiling solvent, e.g. toluene, xylene. The mix is then refluxed at a temperature of 212-350° F., preferably 230-300° F., for a period 40 of 1-10 hours, preferably 2-6 hours in a nitrogen atmosphere in the presence of a catalyst, such as 1-10% (based on the polymer) of a mildly acidic catalyst such as zinc or aluminum chloride. The product is filtered, the solvent and excess amine are removed by evaporation 45 in a vacuum and the polymer is redissolved in the desired solvent. In the reaction, the amine group reacts with the aldehyde or keto group of the polymer, forming water and an azomethine group >C=N—R. The water is removed by distillation or by absorption by the catalyst.

50 The long chain amines employed in this invention are those having from about 8 to about 20 carbon atoms. Among the amines that may be used are tertiary octyl primary amine, tertiary dodecyl primary amine, and Primene 81R which is a mixture of tertiary alkyl 55 primary amines of 15 to 18 carbon atoms.

60 The following examples will serve to illustrate this invention.

## EXAMPLE 1

65 Vinyl acetate, mixed arachidyl behenyl fumarate and cinnamaldehyde in the mole ratio of 1.4/635/365 were dissolved in sufficient benzene to make a 50 percent solution by weight. 1.0 percent of benzoyl peroxide was added and polymerization was conducted at 110° F. for 17 hours in the presence of gamma radiation at a dose rate of 1.15 MR/hr. Then 0.7 mole of tertiary octyl amine was added after benzene had been removed from

3

the mixture by distilling under reduced pressure. The residue was dissolved in approximately 2.5 times its weight of xylene, and refluxed 4.5 hours in a nitrogen atmosphere in the presence of 8.8 percent anhydrous zinc chloride, based on the polymer. This solution was then filtered, the solvent and excess amine were removed under reduced pressure, and the polymer was dissolved in 50 percent of its weight of benzene.

**EXAMPLE 2**

The same procedure as Example 1 was followed, substituting methyl vinyl ketone for the cinnamaldehyde. Mole ratios, concentrations, catalyst and reactions times and temperatures were the same as in Example 1.

**EXAMPLE 3**

Employing the same procedure as in Example 1 a related product was prepared in which crotonaldehyde was substituted for the cinnamaldehyde. Again the same mole ratios, concentrations, catalysts and reaction conditions were used.

#### EXAMPLE 4

A commercial fuel oil was selected for stability tests using the oil itself as well as blends of the oil containing various of the additives described in the foregoing examples. The oil was a blend of 50 percent virgin distillate and 50 percent cracked stock. Typical inspections of this type of oil are as follows:

|                      |       |
|----------------------|-------|
| Gravity, API         | 30-33 |
| Color (Tag Robinson) | 10    |
| Flash, ° F           | 130   |
| Sulfur (percent)     | 1.0   |
| Aniline point, ° F   | 136   |
| Dist. I.B.P. (° F.)  | 315   |
| 10%                  | 392   |
| 50%                  | 479   |
| 90%                  | 581   |
| E.B.P.               | 660   |

To various samples of the fuel oil were added the materials set forth in Table I below. The base fuel and each of the additive blends were subjected to a stability test which consisted in storing the fuel oil for a period of 16 hours while maintaining the temperature at 210° F. At the end of the 16 hours the fuel oil was filtered and the amount of sediment that had been formed during the storage period was quantitatively determined. The color stability of the various fuel oil samples was also determined by measuring the amount of white light that could be transmitted through each of the filtered samples after the storage test relative to the amount of the same white light that could be transmitted through the unheated, uninhibited base fuel.

Table I sets forth the data obtained in these tests:

Table I

#### ACCELERATED STORAGE STABILITY TEST

| Additive                      | Insoluble Sediment Formed After 16 Hours @ 210° F., mg./600 g. Oil | Percent Color Hold * |
|-------------------------------|--------------------------------------------------------------------|----------------------|
| None                          | 12.6                                                               | 71                   |
| 0.01% of Product of Example 1 | 1.4                                                                | 81                   |
| 0.01% of Product of Example 2 | 1.2                                                                | 83                   |
| 0.01% of Product of Example 3 | 0.9                                                                | 82 65                |

\* Percent transmission of white light through filtrate from 16 hour-  
210° F. sediment test, relative to unheated, uninhibited base fuel.

It will be noted from the data in Table I that each of these polymers was very effective in reducing the sediment-forming tendency, as well as preventing degradation of the fuel oil, as indicated by the color hold test.

4

It is not intended that this invention be limited to the specific examples presented by way of illustration. The scope of the invention is limited only by the appended claims.

What is claimed is:

1. A stabilized hydrocarbon oil composition consisting of a major proportion of hydrocarbons boiling in the range of from about 350° F. to about 900° F., and a minor proportion of a reaction product of a long chain tertiary alkyl primary amine with a copolymer of a vinyl ester of a short chain fatty acid, a long chain alcohol ester of a conjugated unsaturated dibasic acid, and a compound selected from the class of alpha, beta unsaturated aldehydes and ketones having the general structure:



20 wherein R is selected from the class consisting of hydro-  
gen, aliphatic groups of from 1 to 8 carbon atoms, phenyl  
groups and alkyl phenyl groups of from 1 to 3 alkyl car-  
bon atoms and R' and R'' are selected from the class  
consisting of hydrogen and aliphatic hydrocarbon groups  
25 of from 1 to 3 carbon atoms, said copolymer being pre-  
pared from monomers in proportion of from about 1 to  
1.5 moles of vinyl ester, from 0.5 to about 0.7 mole of  
the dibasic acid ester and from about 0.3 to 0.5 mole of  
said compound by heating at a temperature in the range  
30 from about 60° F. to 212° F. to produce a copolymer  
having a molecular weight in the range from 1,000 to  
100,000, and said reaction product being prepared by  
heating at a temperature in the range of about 212° F.  
to 350° F. for a period of 1 to 10 hours, 1 to 3 moles  
35 of said amine per one mole of said compound in said  
copolymer, said reaction product being present in said  
hydrocarbon oil composition in an amount sufficient to  
inhibit the formation of sediment in the said oil.

2. Composition as defined by claim 1 wherein the concentration of the reaction product in the hydrocarbon oil composition is within the range of about 0.001% and about 0.2%.

3. Composition as defined by claim 1 wherein the long chain amine has from about 8 to about 20 carbon atoms.

45 4. Composition as defined by claim 1 wherein said reaction product is prepared from tertiary octyl amine and a copolymer of vinyl acetate, mixed arachidyl-behenyl fumarate and methyl vinyl ketone.

5. Composition as defined by claim 1 wherein said  
reaction product is prepared from tertiary octyl amine and  
a copolymer of vinyl acetate, mixed arachidyl-behenyl  
fumarate and crotonaldehyde.

6. Composition as defined by claim 1 wherein said reaction product is prepared from tertiary octyl amine and a copolymer of vinyl acetate, arachidyl-behenyl fumarate and cinnamaldehyde.

**References Cited in the file of this patent**

UNITED STATES PATENTS

|           |                |               |
|-----------|----------------|---------------|
| 2,122,707 | Balthis        | July 5, 1938  |
| 2,353,192 | Sargent et al. | July 11, 1944 |
| 2,387,501 | Dietrich       | Oct. 23, 1945 |
| 2,457,279 | Scott          | Dec. 28, 1948 |
| 2,469,737 | McNab et al.   | May 10, 1949  |
| 2,583,204 | Bevan et al.   | Jan. 22, 1952 |
| 2,737,452 | Catlin et al.  | Mar. 6, 1956  |
| 2,771,348 | Meguerian      | Nov. 20, 1956 |
| 2,793,943 | Moore          | May 28, 1957  |
| 2,800,452 | Bondi et al.   | July 23, 1957 |

## FOREIGN PATENTS

523.748 Belgium Nov. 14, 1953